

H. ABRAHAM.

PROCESS AND APPARATUS FOR THE MANUFACTURE AND PREPARATION OF ROOFING STRIPS.

APPLICATION FILED OCT. 21, 1908.

1,126,932.

Patented Feb. 2, 1915.



Witnesses:

John O. Gempeler  
Emil A. Niedhauer.

Inventor  
Herbert Abraham,  
By his Attorney  
Kenyon & Kenyon.

# UNITED STATES PATENT OFFICE.

HERBERT ABRAHAM, OF BOUND BROOK, NEW JERSEY.

## PROCESS AND APPARATUS FOR THE MANUFACTURE AND PREPARATION OF ROOFING STRIPS.

1,126,932.

Specification of Letters Patent.

Patented Feb. 2, 1915.

Application filed October 21, 1908. Serial No. 458,807.

To all whom it may concern:

Be it known that I, HERBERT ABRAHAM, a citizen of the United States, and a resident of Boundbrook, county of Somerset, and 5 State of New Jersey, have invented certain new and useful Improvements in the Process and Apparatus for the Manufacture and Preparation of Roofing-Strips, of which the following is a specification.

10 My invention relates to the manufacture and preparation of roofing strips and especially comprehends a novel manner of producing improved serrated roofing strips, with a peculiar arrangement of apparatus 15 therefor.

Various and important objects of my invention are, not only to produce serrated roofing strips which have been treated or saturated with a protective compound, but 20 also to produce serrated roofing strips in which the serrated edges as well as the flat surfaces of the strips shall have applied to them a protective or weatherproof coating.

In general it is the object of my invention to provide an arrangement which is 25 conducive to economy and efficiency of operation and construction, and to increase the durability and efficiency of such serrated roofing strips.

30 Further objects, advantages and features will more clearly appear from the detail description given below, taken in connection with the accompanying drawing which forms a part of this specification.

35 In the drawing, Figure 1 is a perspective view showing various parts of one form of a novel apparatus and process which produce my improved roofing strips. Fig. 2 shows a section through the saturating tank.

40 Fig. 3 is a section through one of the coating tanks showing the coating rolls. Fig. 4 is a plan view of a portion of one of my improved roofing strips, and Fig. 5 is a section thereof taken on the line V—V.

45 Referring to Figs. 1 and 2, 1 represents an elongated sheet of roofing material, such as felt, paper, burlap, or other suitable material, but preferably of felt. The sheet 1 is guided through the saturating or impreg-

In the tank 2 is a compound 4 rendered fluid by means of heat which is designed to saturate or impregnate the sheet 1 and to protect it from elemental and other deteriorating actions. Within the tank 2 are steam 55 pipes 20 which properly heat the compound 4 so that it is easily and readily absorbed by the sheet 1. For the sake of clearness the impregnating material 4, steam pipes 20 are omitted in Fig. 1. These are, however, 60 clearly shown in Fig. 2. The saturating or impregnating compound 4 preferably consists of a soft non-hardening compound containing resins, oils, fats, waxes, bitumens, tars, pitches or their equivalents, either 65 singly or in combination. It is not to be understood, however, that this is the only form of saturation that may be employed, for any compound which will render the fabric waterproof and pliable may likewise be used 70 to advantage.

After leaving the tank 2 and guiding rolls 3 the sheet 1 is carried to cutting rolls 5 one of which possesses a zigzag cutter 6. The cutter 6 is arranged to cut a zigzag or other 75 path through the sheet 1, splitting it longitudinally into two roofing strips 7 and 8, each with serrations or notches 9. From the cutting rolls the strip 7 is carried upward to the coating or facing rolls 10 which operate 80 to apply a coating or facing material from the pan 11 to the strip. At the same time the strip 8 is carried downward to similar coating or facing rolls 12 and pan 13. The coating rolls 10 and 12 take up on their surfaces the melted coating compound or facing material 14 from the pans 11 and 13 and apply it to the strips 7 and 8 (see also Fig. 3). The pans 11 and 13 are provided with steam pipes 19 to heat the compound 14 so 90 that it will be fluid enough to be properly applied to the strips. For the sake of clearness the compound 14 and the steam pipes 19 are omitted from Fig. 1, but are clearly shown in Fig. 3.

95 Adjacent to the coating or facing rolls are troughs 16 which feed the hot facing compound 14 to the tops of the strips 7 and 8. The hot compound 14 is fed to the troughs 16 by supply tubes 17 from any suitable 100

source. The compound 14 is deposited by the troughs 16 in the center of the strips 7 and 8 and beneath the upper rolls 10 and 12. This is clearly shown in Fig. 3. The upper rolls 10 and 12 spread the coating or facing over the upper surface of the strips and incidentally both edges of the strips 7 and 8 and especially the serrated edges 9 of said strips have the proper amount of this coating applied to them. The facing material or compound 14 is preferably of a harder consistency than that used in the tank 2 for impregnating, and it may consist of one or more of the ingredients mentioned in connection with the latter, viz, materials of a resinous, fatty, waxy, bituminous, tarry or pitchy nature; or it may be composed of the particular ingredients set forth in United States Patent No. 775,635 or 775,636.

20 After leaving the coating rolls 10 and 12 the strips are coiled into rolls or otherwise conveniently put up in marketable shape. If desired the roofing strips may be surfaced with powdered soapstone or other material 25 to prevent them from sticking together when rolled or otherwise packed.

Referring to Figs. 4 and 5, I show a portion of the serrated roofing strip 8 with the serrations or notches 9 thereon. In these figures various of the dimensions have been greatly exaggerated in order to clearly show that the coating 15 from the coating rolls 12 is applied to the edges as well as to one of the flat surfaces of the strip.

35 By the above method and means, in which the firm, pliable, waterproof and weatherproof coating 14 is applied after the sheet 1 is cut into the strips 7 and 8, serrated roofing strips are produced in which the 40 edges, and especially the serrated edges, are fully protected from the detrimental action of the weather and other causes. The coating or facing 15 not only protects the edges of the strips from the detrimental action of 45 water and the climate but also reinforces the edges and prevents them from cracking, swelling, etc. This is especially important since it is usually the serrated edges which lie exposed and are more liable to deteriorate or become damaged. By my improvements 50 I also produce two serrated strips with only one cutter and the whole arrangement is conducive to economy and efficiency of operation and construction.

55 Although I have described my improvements in great detail, I do not limit myself to such details, but,

Having fully and clearly set forth my invention what I claim as new and desire to 60 secure by Letters Patent, is:

1. The improved process for producing flexible waterproof roofing strips which consists in impregnating a web of suitable ma-

terial with a protective weatherproofing compound, cutting the impregnated web 65 into strips and then coating the strips with a protective weatherproofing substance so that the coating will be applied to the cut edges thereof.

2. The improved process for producing 70 serrated roofing strips which consists in impregnating a web of sheet material with a protective compound, cutting the impregnated web into serrated strips and then facing the strips with a protective weather- 75 proofing substance so that the facing will be applied to the cut edges thereof.

3. The improved process for producing serrated flexible waterproof roofing strips which consists in impregnating a web of 80 sheet material with an asphaltic composition, cutting said impregnated web into serrated strips and then coating said strips with a coating of asphaltic or bituminous material so that the coating will be applied 85 to the cut edges of the strips.

4. The improved process for producing serrated flexible waterproof roofing strips which consists in impregnating a web of 90 suitable material with a waterproofing compound, cutting said web into impregnated strips and then facing said strips with a waterproofing compound so that the facing will be applied to the cut edges of the strips.

5. The improved process for producing 95 serrated flexible waterproof roofing strips which consists in cutting a web of suitable material into strips with serrated edges and then simultaneously facing said strips with a protective weatherproofing coating so that the coating will be applied to the cut serrated edges of said strips.

6. In a machine of the class described, the combination of means for cutting a zigzag path through a sheet of suitable material 105 to form serrated strips, means for applying a protective weatherproofing coating to the lower faces of said strips and means for applying a protective coating to the upper faces of said strips, said means being arranged to also apply said coating to the edges of said strips.

7. The improved process of producing flexible weatherproof roofing which consists in impregnating a strip of suitable material 115 with a protective weatherproofing compound, cutting an edge of the impregnated weatherproof strip so as to form serrations or notches along the edge and then coating the cut edges of the serrations or notches 120 with a protective weatherproofing substance.

8. The improved process of producing flexible weatherproof roofing which consists in impregnating a strip of suitable material with a protective weatherproofing com- 125 pound, cutting an edge of the weatherproof

strip so as to form serrations or notches along the edge and then coating the cut edges of the serrations or notches with a protective weatherproofing substance of a harder consistency than that of the impregnating compound.

In testimony whereof, I have signed my

name to this specification, in the presence of two subscribing witnesses.

HERBERT ABRAHAM.

Witnesses:

H. F. RUGEN,

Jos L. DURN.

It is hereby certified that in Letters Patent No. 1,126,932, granted February 2, 1915, upon the application of Herbert Abraham, of Boundbrook, New Jersey, for an improvement in "Processes and Apparatus for the Manufacture and Preparation of Roofing-Strips," an error appears in the printed specification requiring correction as follows: Page 2, lines 62, 79, 88, and 96, for the word "waterproof" read *weatherproof*; and that the said Letters Patent should be read with this correction therein that the same may conform to the record of the case in the Patent Office.

Signed and sealed this 16th day of March, A. D., 1915.

[SEAL.]

J. T. NEWTON,

*Acting Commissioner of Patents.*